



US012104297B1

(12) **United States Patent**  
**Waldman et al.**

(10) **Patent No.:** US 12,104,297 B1  
(b4) **Date of Patent:** Oct. 1, 2024

(54) **CHEMICAL RESISTANT FABRIC**(71) Applicant: **Global Trademarks, Inc.**, Easton, PA (US)(72) Inventors: **Mark Waldman**, New Hope, PA (US); **Ruth Gordon**, Bernardsville, NJ (US)(73) Assignee: **Global Trademarks, Inc.**

(\* ) Notice: Subject to any disclaimer, the term of this patent is extended or adjusted under 35 U.S.C. 154(b) by 126 days.

(21) Appl. No.: **17/591,667**(22) Filed: **Feb. 3, 2022****Related U.S. Application Data**

(60) Provisional application No. 63/145,020, filed on Feb. 3, 2021.

(51) **Int. Cl.****D04B 21/16** (2006.01)(52) **U.S. Cl.**CPC ..... **D04B 21/16** (2013.01); **D10B 2401/061** (2013.01); **D10B 2501/04** (2013.01)(58) **Field of Classification Search**

CPC ..... D04B 21/06; D04B 21/16; D04B 21/18; D10B 2501/04; D10B 2401/061

USPC ..... 66/192, 193, 195  
See application file for complete search history.(56) **References Cited**

## U.S. PATENT DOCUMENTS

519,101 A \* 5/1894 Spooner ..... D04B 21/18  
D5/47  
752,033 A \* 2/1904 Clewley ..... D04B 21/10  
66/193

|               |          |                 |
|---------------|----------|-----------------|
| 1,931,822 A   | 4/1933   | Hoffman         |
| 2,060,689 A   | 10/1935  | Read            |
| 2,136,367 A * | 11/1938  | Amidon .....    |
|               |          | D04B 21/18      |
|               | 66/192   |                 |
| 2,149,032 A * | 2/1939   | Schonfeld ..... |
|               |          | D04B 21/18      |
|               | 66/84 R  |                 |
| 2,153,645 A * | 4/1939   | Schonfeld ..... |
|               |          | D04B 21/18      |
|               | 66/192   |                 |
| 2,183,108 A * | 12/1939  | Schonfeld ..... |
|               |          | D04B 21/18      |
|               | 66/192   |                 |
| 2,199,449 A * | 5/1940   | Schonfeld ..... |
|               |          | D04B 21/18      |
|               | 66/203   |                 |
| 2,267,578 A * | 12/1941  | Schonfeld ..... |
|               |          | D04B 23/22      |
|               | 66/203   |                 |
| 2,289,302 A * | 7/1942   | Bradshaw .....  |
|               |          | D04B 21/18      |
|               | 66/195   |                 |
| 2,323,396 A * | 7/1943   | Hayto .....     |
|               |          | D04B 1/18       |
|               | 66/195   |                 |
| 2,411,175 A * | 11/1946  | Wagler .....    |
|               |          | D04B 21/18      |
|               | 66/193   |                 |
| 2,800,783 A * | 7/1957   | Abood .....     |
|               |          | D04B 21/08      |
|               | 66/84 R  |                 |
| 2,910,853 A * | 11/1959  | Howard .....    |
|               |          | D04B 21/18      |
|               | 66/172 R |                 |

(Continued)

*Primary Examiner* — Danny Worrell(74) *Attorney, Agent, or Firm* — BELLES KATZ LLC(57) **ABSTRACT**

Described herein is a fabric having a warp knit construction comprising a first yarn forming a plurality of stitches, the first yarn being a hard yarn and having a first denier ranging from about 20 to about 150, a second yarn in-laid through the first yarn, the second yarn being an elastomeric yarn and having a second denier ranging from about 210 to about 450; and, wherein the first yarn is present in an amount ranging from about 90 wt. % to about 99 wt. % based on the total weight of the fabric, and wherein the second yarn is present in an amount ranging from about 1 wt. % to about 10 wt. % based on the total weight of the fabric.

**20 Claims, 7 Drawing Sheets**

| (56)                  | References Cited        |                        |                   |                            |                        |
|-----------------------|-------------------------|------------------------|-------------------|----------------------------|------------------------|
| U.S. PATENT DOCUMENTS |                         |                        |                   |                            |                        |
| 2,960,855 A *         | 11/1960 Siciliano ..... | D04B 21/18<br>450/156  | 4,103,485 A *     | 8/1978 Brues .....         | D04B 21/18<br>66/192   |
| 2,992,550 A *         | 7/1961 Frith, Jr. ..... | D04B 21/10<br>66/195   | 4,377,007 A       | 3/1983 Sudjian             |                        |
| 3,077,758 A *         | 2/1963 Siciliano .....  | D04B 21/12<br>2/DIG. 9 | 4,528,699 A       | 7/1985 Hughes              |                        |
| 3,084,529 A *         | 4/1963 Scheibe .....    | D04B 21/10<br>66/193   | 4,748,078 A *     | 5/1988 Doi .....           | D04B 21/08<br>66/169 A |
| 3,106,079 A *         | 10/1963 Kohl .....      | D04B 21/18<br>66/193   | 5,083,316 A       | 1/1992 Kuehner et al.      |                        |
| 3,183,685 A *         | 5/1965 Riehl .....      | D04B 21/12<br>66/193   | 5,184,968 A       | 2/1993 Michalochick et al. |                        |
| 3,672,187 A *         | 6/1972 Simpson .....    | D04B 21/165<br>66/192  | 5,359,732 A       | 11/1994 Waldman et al.     |                        |
| 3,691,796 A *         | 9/1972 Mayer .....      | D04B 21/00<br>66/193   | 6,758,068 B2 *    | 7/2004 Shirasaki .....     | D04B 21/16<br>66/170   |
| 3,733,859 A *         | 5/1973 Wittmann .....   | D04B 21/12<br>66/193   | 7,465,683 B2      | 12/2008 McMurray           |                        |
| 3,910,075 A           | 10/1975 Holliday .....  | D04B 21/18             | 7,727,286 B2      | 6/2010 Reid et al.         |                        |
| 3,922,888 A *         | 12/1975 Patterson ..... | D04B 21/18<br>D5/47    | 8,322,168 B2 *    | 12/2012 Wall .....         | D04B 21/18<br>66/193   |
| 4,074,543 A *         | 2/1978 Schmidt .....    | D04B 21/12<br>66/193   | 8,726,700 B2      | 5/2014 Waldman et al.      |                        |
|                       |                         |                        | 8,769,718 B2      | 7/2014 Riehl               |                        |
|                       |                         |                        | D806,359 S        | 1/2018 Waldman             |                        |
|                       |                         |                        | 9,896,790 B2 *    | 2/2018 Ko .....            | D03D 19/00             |
|                       |                         |                        | 2007/0174972 A1   | 8/2007 Carney et al.       |                        |
|                       |                         |                        | 2010/0229605 A1 * | 9/2010 Keitch .....        | D04B 21/12<br>66/193   |
|                       |                         |                        | 2012/0297840 A1   | 11/2012 Yeung              |                        |
|                       |                         |                        | 2016/0122907 A1   | 5/2016 Liu et al.          |                        |
|                       |                         |                        | 2019/0309452 A1   | 10/2019 Liao et al.        |                        |

\* cited by examiner



FIG. 1



FIG. 2



FIG. 3



FIG. 4



FIG. 5



FIG. 6



FIG. 7

## 1

## CHEMICAL RESISTANT FABRIC

CROSS-REFERENCE TO RELATED  
APPLICATIONS

The present application claims the benefit of priority to U.S. Provisional Patent Application Ser. No. 63/145,020, filed on Feb. 3, 2021, the entirety of which is incorporated herein by reference.

## BACKGROUND

Stretch fabrics have many applications in active wear, which expose these materials to conditions that may not be suitable for prolonged deformation and recovery in such stretch fabrics—such as chlorinated pools. Therefore, a need exists for a new stretch fabric that is suitable for such active wear applications, and which can exhibit the necessary prolonged recovery characteristics that are needed for such applications.

## BRIEF SUMMARY

In some embodiments, the present invention is directed to a fabric having a warp knit construction comprising: a repeating array of cells, each cell defined by an inlay yarn; a plurality of stitches formed inside of each cell, the plurality of stitches formed by a hard yarn; and wherein the number of stitches per cell ranges from about 20 to about 300.

Other embodiments of the present invention include a fabric having a warp knit construction comprising: a first yarn forming a plurality of stitches extending along in a knit direction, the first yarn having a first denier; a second yarn in-laid through the first yarn, the second yarn extending along the knit direction and having a repeating pattern that extends across at least 4 wales for every 4 courses, the second yarn having a second denier; and wherein a ratio of the second denier to the first denier ranges from about 2:1 to about 15:1.

Other embodiments of the present invention include a fabric having a warp knit construction comprising: a first yarn forming a plurality of stitches, the first yarn being a hard yarn and having a first denier ranging from about 20 to about 150; a second yarn in-laid through the first yarn, the second yarn being an elastomeric yarn and having a second denier ranging from about 210 to about 450; and wherein the first yarn is present in an amount ranging from about 90 wt. % to about 99 wt. % based on the total weight of the fabric, and wherein the second yarn is present in an amount ranging from about 1 wt. % to about 10 wt. % based on the total weight of the fabric.

Other embodiments of the present invention include a fabric having a warp knit construction, the fabric having a first major surface opposite a second major surface, the warp knit construction comprising: a repeating array of cells, each cell having a perimeter that is defined by an inlay yarn; a repeating array of central regions, each central region located inside of the perimeter of each cell, and each central region comprising a plurality of stitches that are formed by a hard yarn; and wherein in a first state, no external stress is applied to the fabric and in a second state, external stress is applied to the fabric in a direction substantially parallel to each of the first major surface and the second major surface; and wherein in the first state the repeating array of central regions exhibit a thickness ranging from about 60 mils to about 120 mils, as measured between the first major surface and the second major surface of the fabric, and wherein in

## 2

the second state, the repeating array of central regions exhibit a thickness ranging from about 10 mils to about 30 mils, as measured between the first major surface and the second major surface of the fabric.

5 Other embodiments of the present invention include a swimsuit comprising the aforementioned fabric.

Other embodiments of the present invention include a method of knitting a fabric comprising: knitting a first yarn to form a plurality of stitches that extends in a vertical direction, the first yarn having a first denier; in-laying a second yarn with the first yarn such that the second yarn extends along the vertical direction and has a repeating pattern that extends across at least 4 wales for every 4 courses, the second yarn having a second denier; and wherein a ratio of the second denier to the first denier ranges from about 2:1 to about 15:1.

Further areas of applicability of the present invention will become apparent from the detailed description provided hereinafter. It should be understood that the detailed description and specific examples, while indicating the preferred embodiment of the invention, are intended for purposes of illustration only and are not intended to limit the scope of the invention.

## BRIEF DESCRIPTION OF THE DRAWINGS

The present invention will become more fully understood from the detailed description and the accompanying drawings, wherein:

30 FIG. 1 is a perspective view of the fabric of the present invention;

FIG. 2 is a close-up view of the first major surface of the fabric in region II shown in FIG. 1;

FIG. 3 is a close-up view of the second major surface of the fabric in region II shown in FIG. 1;

FIG. 4 is a cross-sectional view of the fabric along line V-V shown in FIG. 3;

FIG. 5 is a stitch diagram of the knit pattern of the fabric of the present invention having a first yarn and a second yard;

FIG. 6 is a stitch diagram view of the first yarn shown in FIG. 5; and

FIG. 7 is a view of the second yarn only, as shown in FIG. 5, for demonstrative purposes.

## DETAILED DESCRIPTION

The following description of the preferred embodiment(s) is merely exemplary in nature and is in no way intended to limit the invention, its application, or uses.

As used throughout, ranges are used as shorthand for describing each and every value that is within the range. Any value within the range can be selected as the terminus of the range. In addition, all references cited herein are hereby incorporated by reference in their entireties. In the event of a conflict in a definition in the present disclosure and that of a cited reference, the present disclosure controls.

Unless otherwise specified, all percentages and amounts expressed herein and elsewhere in the specification should be understood to refer to percentages by weight. The amounts given are based on the active weight of the material.

The description of illustrative embodiments according to principles of the present invention is intended to be read in connection with the accompanying drawings, which are to be considered part of the entire written description. In the description of embodiments of the invention disclosed

herein, any reference to direction or orientation is merely intended for convenience of description and is not intended in any way to limit the scope of the present invention. Relative terms such as "lower," "upper," "horizontal," "vertical," "above," "below," "up," "down," "top," and "bottom" as well as derivatives thereof (e.g., "horizontally," "downwardly," "upwardly," etc.) should be construed to refer to the orientation as then described or as shown in the drawing under discussion. These relative terms are for convenience of description only and do not require that the apparatus be constructed or operated in a particular orientation unless explicitly indicated as such.

Terms such as "attached," "affixed," "connected," "coupled," "interconnected," and similar refer to a relationship wherein structures are secured or attached to one another either directly or indirectly through intervening structures, as well as both movable or rigid attachments or relationships, unless expressly described otherwise. Moreover, the features and benefits of the invention are illustrated by reference to the exemplified embodiments. Accordingly, the invention expressly should not be limited to such exemplary embodiments illustrating some possible non-limiting combination of features that may exist alone or in other combinations of features; the scope of the invention being defined by the claims appended hereto.

Unless otherwise specified, all percentages and amounts expressed herein and elsewhere in the specification should be understood to refer to percentages by weight. The amounts given are based on the active weight of the material. According to the present application, the term "about" means  $\pm 5\%$  of the reference value. According to the present application, the term "substantially free" less than about 0.1 wt. % based on the total of the referenced value.

FIGS. 1-4 shows a fabric 1 according to the present invention. The fabric 1 may be a warp knit fabric. The term 'warp knit fabric' refers to the fabric 1 having a warp knit construction 10. According to the present invention, the warp knit construction 10 refers to a knit that is different from a weft knit construction (such as flatbed knits and circular knits). The warp knit construction 10 of the present invention may be a raschel knit that is formed along a knit direction KD using a raschel knitting machine.

The fabric 1 may comprise a front major surface 2 (also referred to as the "technical back") opposite a rear major surface 3 (also referred to as the "technical face"). The front major surface 2 of the fabric 1 may comprise a plurality of protrusions 50 that are offset by a plurality of intersecting channels 60. Each of the protrusions 50 may extend outward from the plurality of intersecting channels 60 in a direction extending from the rear major surface 3 toward the front major surface 2 of the fabric 1. The protrusions 50 may terminate at an apex 51 that is vertically offset from a floor 61 of the intersecting channels 60 by a non-zero value. The protrusions 50 may terminate at an apex 51 that is vertically offset from a floor 61 of the intersecting channels 60 by a distance of at least 5 mils.

The front major surface 2 of the fabric 1 may comprise the apex 51 of the protrusion 50, the floor 61 of the intersecting channels 60, and the exposed surface extending there-between, thereby forming a first topography for the front major 2.

The rear major surface 3 of the fabric 1 may comprise a plurality of recesses 70 that are offset from each other by a plurality of intersecting walls 80. Each of the recesses 70 may extend inward from the plurality of intersecting walls 80 in a direction extending from the rear major surface 3 toward the front major surface 2 of the fabric 1. The recesses

70 may terminate at a recess floor 71 that is vertically offset from a top 81 of the intersecting walls 80 by a non-zero value. The recesses 70 may terminate at a recess floor 71 that is vertically offset from a top 81 of the intersecting walls 80 by a distance of at least 5 mils.

The rear major surface 3 of the fabric 1 may comprises the top 81 of the intersecting walls 80, the plurality of recess floors 71, and the exposed surface extending there-between, thereby forming a second topography for the rear major surface 3. The first topography and the second topography are different. The first topography and the second topography may be negatives of each other.

The fabric 1 may exhibit a fabric thickness  $t_F$  as measured by the distance between the apex 51 of the protrusion 50 and the top 81 of the intersection walls 80. In a first state where no external stress is applied to the fabric 1, the fabric thickness  $t_F$  may range from about 60 mils to about 120 mils—including all thicknesses and sub-ranges there-between. In a second state where external stress is applied in a direction that is substantially parallel to each of the front major surface 2 and the rear major surface 3—thereby stretching the fabric 1 along a plane substantially parallel to each of the front major surface 3 and the rear major surface 3—the fabric thickness  $t_F$  may range from about 10 mils to about 30 mils—including all thicknesses and sub-ranges there-between.

In the first state, two adjacent apex 510 of two immediately adjacent protrusions 50 along first direction may be offset by a first distance  $D_1$  that ranges from about 140 mils to about 250 mils—including all thicknesses and sub-ranges there-between. In the second state, the first distance  $D_1$  may be a value of at least 300% the value of  $D_1$  in the first state—including all thicknesses and sub-ranges there-between. The first direction may be parallel to a knit direction or may be substantial orthogonal to the knit direction (as discussed in greater detail herein).

Referring now to FIGS. 5-7, a raschel knit may be formed in line with the movement of the needles along the knit direction KD. In a non-limiting example, the stitch diagram of FIGS. 5-7 may demonstrate how a warp knit construction 10 may be formed having two different yarns that are interconnected by cross stitches.

Referring to FIGS. 5-7, in particular, the warp knit construction 10 may be formed of a first yarn 100 (also referred to as a "first thread") and a second yarn 200 (also referred to as a "second thread"). The first yarn 100 may be different from the second yarn 200. In a preferred embodiment, the first yarn 100 is different from the second yarn 200.

As described in greater detail herein, the first yarn 100 may be a hard yarn (also referred to as an "inelastic yarn"), and the second yarn 200 may be an elastomeric yarn. The term "elastomeric yarn" refers to a yarn capable of deforming (e.g. elongating) from a first state to a second state under an applied stress and recovering to the first state from the second state once the applied stress is removed. The first state may be a first set of dimensions and the second state may be a second set of dimensions that are greater than the first set of dimensions in at least one direction (length, width, thickness). The term "hard yarn" refers to a yarn either not capable of deforming from the first state to the second state under an applied stress (i.e., the yarn either does not change dimensions or the yarn breaks under the applied stress) or refers to a yarn that transitions from the first state to the second state but does not exhibit recovery from the second state back to the first state once the applied stress is removed.

The warp knit construction 10 may comprise a plurality of stitches that are each formed by an interlocking knit loop 110

that is created by a needle **20** during knitting—whereby the travel along the needles **20** control the path of each of the first yarn **100** and the second yarn **200** within the warp knit construction **10**. Each stitch may be represented by each knit loop **110** shown on the stitch diagram of FIGS. 5-6.

Referring to FIGS. 2-7, each protrusion **50** of the first major surface **2** may be formed by the first yarn **100**. The apex **51** of each protrusion **50** may be formed from the first yarn **100**. Each protrusion **50** of the first major surface **2** may be substantially free of the second yarn **200**. The apex **51** of each protrusion **50** may be substantially free of the second yarn **200**.

Each of the intersecting channels **60** of the first major surface **2** may comprise the second yarn **200**. The floor **61** of each intersecting channel **60** may comprise the second yarn **200**. Each of the intersecting channels **60** of the first major surface **2** may comprise the first yarn **100**. The floor **61** of each intersecting channel **60** may comprise the first yarn **100**.

Each recess **70** of the second major surface **3** may be formed by the first yarn **100**. The floor **71** of each recess **70** may be formed from the first yarn **100**. Each recess **70** of the second major surface **3** may be substantially free of the second yarn **200**. The floor **71** of each recess **70** may be substantially free of the second yarn **200**.

Each of the intersecting walls **80** of the second major surface **3** may comprise the second yarn **200**. The top **81** of each intersecting wall **80** may comprise the second yarn **200**. Each of the intersecting walls **80** of the second major surface **3** may comprise the first yarn **100**. The top **81** of each intersecting wall **80** may comprise the first yarn **100**.

The warp knit construction **10** may comprise a plurality of stitches, each stitch formed by the knit loop **110** of the first yarn **100**, whereby a portion **115** of the first yarn **100** spans between the knit loops **110**. The warp knit construction **10** may comprise a repeating array of cells **210** formed by the second yarn **200**. Each cell **210** may be defined by a perimeter **215**, whereby the perimeter **215** is formed by the second yarn **200**. The perimeter **215** of each cell **210** may define a central region **CR** located entirely within the perimeter **215** of each cell **210**. The perimeter **215** of each cell **210** may be a closed-perimeter. The plurality of cells **210** may define an array of central regions **CR** located inside of the plurality of cells **210**.

Each cell **210** may be formed by the second yarn **200**, whereby the second yarn **200** is an inlay yarn trapped within the warp knit construction **10** by the first yarn **100** that span across the entirety of the warp knit construction **10**. The central region **CR** may be occupied the plurality of stitches. The central region **CR** may be occupied solely by the plurality of stitches. The central region **CR** may be occupied solely by the first yarn **100**. The central region **CR** may be substantially free of the second yarn **200**.

According to the present invention, a plurality of stitches of the first yarn **100** may be located within a single cell **210** of the second yarn **200**. The number of stitches of the first yarn **100** located inside the perimeter **215** of a single cell **210** may range from about 20 to about 300—including all individual integers and sub-ranges there-between. In some embodiments, the number of stitches of the first yarn **100** located inside the perimeter **215** of a single cell **210** may range from about 40 to about 250—including all individual integers and sub-ranges there-between. In some embodiments, the number of stitches of the first yarn **100** located inside the perimeter **215** of a single cell **210** may range from about 45 to about 200—including all individual integers and sub-ranges there-between.

The perimeter of each cell **210** may be collectively formed by a combination of a first one **200a** of the second yarn **200** and a second one **200b** of the second yarn **200**. Each of the first one **200a** and the second one **200b** of the second yarn **200** may be separate threads of the second yarn **200**. Each of the first one **200a** and the second one **200b** of the second yarn **200** may be separate yarns. Independently, each of the first one **200a** and the second one **200b** may not be a bicomponent yarn.

Each one of the first one **200a** and the second one **200b** of the second yarn **200** may span along the knit direction **KD** in a repeating pattern across the courses **C<sub>#</sub>-C<sub>#</sub>** and wales **W<sub>#</sub>-W<sub>#</sub>** formed by the plurality of stitches of the first yarn **100**. In a non-limiting embodiment, the first one **200a** and the second one **200b** of the second yarn **200** may overlap at a plurality of overlap points **220** to form the perimeter **215** of the cell **210**. In a non-limiting embodiment, the first one **200a** and the second one **200b** of the second yarn **200** may overlap at a plurality of overlap points **220** to form the closed-perimeter **215** of the cell **210**.

As demonstrated by FIGS. 5 and 7, the first one **200a** of the second yarn **200** may be in-laid in a repeating pattern having a first repeating unit and the second one **200b** of the second yarn **200** may be in-laid in a repeating pattern having a second repeating unit.

The first repeating unit of the first one **200a** of the second yarn **200** may follow a first path **FP<sub>1</sub>** along the knit direction **KD** that spans a first plurality of wales and a first plurality of courses followed by a second path **SP<sub>1</sub>** that follows the knit direction **KD** and spans a second plurality of wales and a second plurality of courses.

The first plurality of wales and the first plurality of courses for the first path **FP<sub>1</sub>** of the first repeating unit may be equal. The first plurality of courses for the first path **FP<sub>1</sub>** of the first repeating unit and the second plurality of courses for the second path **SP<sub>1</sub>** of the first repeating unit may be equal. The first plurality of wales for the first path **FP<sub>1</sub>** of the first repeating unit and the second plurality of wales for the second path **SP<sub>1</sub>** of the first repeating unit may have opposite values, thereby causing the first one **200a** of the second yarn **200** to return to the same wale from which the repeating unit started. For instance, the first plurality of wales of the first path **FP<sub>1</sub>** of the first repeating unit may be equal to six (6) and the second plurality of wales for the second path **SP<sub>1</sub>** of the first repeating may be equal to negative six (-6).

The first plurality of wales for the first path **FP<sub>1</sub>** of the first repeating unit may range from about 3 to about 30—including all integers and sub-ranges there-between. In some embodiments, the first plurality of wales for the first path **FP<sub>1</sub>** of the first repeating unit may range from about 5 to about 30—including all integers and sub-ranges there-between. In some embodiments, the first plurality of wales for the first path **FP<sub>1</sub>** of the first repeating unit may range from about 10 to about 30—including all integers and sub-ranges there-between.

The first plurality of courses for the first path **FP<sub>1</sub>** of the first repeating unit may range from about 3 to about 30—including all integers and sub-ranges there-between. In some embodiments, the first plurality of courses for the first path **FP<sub>1</sub>** of the first repeating unit may range from about 5 to about 30—including all integers and sub-ranges there-between. In some embodiments, the first plurality of courses for the first path **FP<sub>1</sub>** of the first repeating unit may range from about 10 to about 30—including all integers and sub-ranges there-between.

The second plurality of wales for the second path **SP<sub>1</sub>** of the first repeating unit may range from about 3 to about

30—including all integers and sub-ranges there-between. In some embodiments, the second plurality of wales for the second path  $SP_1$  of the first repeating unit may range from about 5 to about 30—including all integers and sub-ranges there-between. In some embodiments, the second plurality of wales for the second path  $SP_1$  of the first repeating unit may range from about 10 to about 30—including all integers and sub-ranges there-between.

The second plurality of courses for the second path  $SP_1$  of the first repeating unit may range from about 3 to about 30—including all integers and sub-ranges there-between. In some embodiments, the second plurality of courses for the second path  $SP_1$  of the first repeating unit may range from about 5 to about 30—including all integers and sub-ranges there-between. In some embodiments, the second plurality of courses for the second path  $SP_1$  of the first repeating unit may range from about 10 to about 30—including all integers and sub-ranges there-between.

The second repeating unit of the second one  $200b$  of the second yarn  $200$  may follow a first path  $FP_2$  along the knit direction  $KD$  that spans a first plurality of wales and a first plurality of courses followed by a second path  $SP_2$  that follows the knit direction  $KD$  and spans a second plurality of wales and a second plurality of courses.

The first plurality of wales and the first plurality of courses for the first path  $FP_2$  of the second repeating unit may be equal. The first plurality of courses for the first path  $FP_2$  of the second repeating unit and the second plurality of courses for the second path  $SP_2$  of the second repeating unit may be equal. The first plurality of wales for the first path  $FP_2$  of the second repeating unit and the second plurality of wales for the second path  $SP_2$  of the second repeating unit may have opposite values, thereby causing the second one  $200b$  of the second yarn  $200$  to return to the same wale from which the repeating unit started. For instance, the first plurality of wales of the first path  $FP_2$  of the second repeating unit may be equal to negative six ( $-6$ ) and the second plurality of wales for the second path  $SP_2$  of the second repeating may be equal to six ( $6$ ).

The first plurality of wales for the first path  $FP_2$  of the second repeating unit may range from about 3 to about 30—including all integers and sub-ranges there-between. The first plurality of wales for the first path  $FP_2$  of the second repeating unit may range from about 5 to about 30—including all integers and sub-ranges there-between. The first plurality of wales for the first path  $FP_2$  of the second repeating unit may range from about 10 to about 30—including all integers and sub-ranges there-between.

The first plurality of courses for the first path  $FP_2$  of the second repeating unit may range from about 3 to about 30—including all integers and sub-ranges there-between. The first plurality of courses for the first path  $FP_2$  of the second repeating unit may range from about 5 to about 30—including all integers and sub-ranges there-between. The first plurality of courses for the first path  $FP_2$  of the second repeating unit may range from about 10 to about 30—including all integers and sub-ranges there-between.

The second plurality of wales for the second path  $SP_2$  of the second repeating unit may range from about 3 to about 30—including all integers and sub-ranges there-between. In some embodiment, the second plurality of wales for the second path  $SP_2$  of the second repeating unit may range from about 5 to about 30—including all integers and sub-ranges there-between. In some embodiments, the second plurality of wales for the second path  $SP_2$  of the second repeating unit may range from about 10 to about 30—including all integers and sub-ranges there-between.

The second plurality of courses for the second path  $SP_2$  of the second repeating unit may range from about 3 to about 30—including all integers and sub-ranges there-between. In some embodiments, the second plurality of courses for the second path  $SP_2$  of the second repeating unit may range from about 5 to about 30—including all integers and sub-ranges there-between. In some embodiments, the second plurality of courses for the second path  $SP_2$  of the second repeating unit may range from about 10 to about 30—including all integers and sub-ranges there-between.

The warp knit construction  $10$  may be formed by knitting the first yarn  $100$  on a first needle bar to form a plurality of knit loops  $110$  that span along a vertical direction between a first number of wales—whereby the first number of wales may range from about 2 to about 4, preferably from about 2 to about 3, including all integers and sub-ranges there-between—and in-laying the second yarn  $200$  with the first yarn  $100$  such that the second yarn  $200$  may extend along the vertical direction and has a repeating pattern that extends across at least 4 different wales for every 4 courses. In some embodiments, the second yarn  $200$  may extend along the vertical direction and have a repeating pattern that extends across at least 5 different wales for every 5 courses.

In a non-limiting example, the first one  $200a$  of the second yarn  $200$  may have a first repeating unit such that the first one  $200a$  of the second yarn  $200$  follows a first path  $FP_1$  along the knit direction  $KD$  that spans from a sixth wale to a first wale (i.e., first plurality of wales of the first repeating unit) and spans from a first course to a sixth course (i.e., first plurality of courses of the first repeating unit) followed by a second path  $SP_1$  that follows along the knit direction  $KD$  and spans from the first wale back to the sixth wale (i.e., second plurality of wales of the first repeating unit) and spans from the sixth course to an eleventh course (i.e., second plurality of courses of the first repeating unit). According to this non-limiting example, the second one  $200b$  of the second yarn  $200$  may have a second repeating unit such that the second one  $200b$  of the second yarn  $200$  follows a first path  $FP_2$  along the knit direction  $KD$  that spans from the sixth wale to an eleventh wale (i.e., first plurality of wales of the second repeating unit) and spans from the first course to the sixth course (i.e., first plurality of courses of the second repeating unit) followed by a second path  $SP_2$  that follows along the knit direction  $KD$  and spans from the eleventh wale back to the sixth wale (i.e., second plurality of wales of the second repeating unit) and spans from the sixth course to an eleventh course (i.e., second plurality of courses of the second repeating unit). The overlap between the first one  $200a$  and the second one  $200b$  at the first course and sixth wale as well as the overlap at the eleventh course and sixth wale forms the perimeter  $215$  of the cell  $210$ .

The present invention is not limited to a value of six ( $6$ ) for such first and second plurality of courses and wales. Thus, the previous example may further apply to first ones  $200a$  and second ones  $200b$  of the second yarn  $200$  when the first and second plurality of courses and wales span the aforementioned ranges.

Each individual cell  $210$  of the warp knit construction  $10$  may have a perimeter  $215$  that spans from about 5 to about 50 courses along the knit direction  $KD$ —including each integer value and sub-range there-between. Each individual cell  $210$  of the warp knit construction  $10$  may have a perimeter  $215$  that spans from about 5 to about 50 wales in a direction transverse to the knit direction  $KD$ —including each integer value and sub-range there-between.

The warp knit construction  $10$  of the fabric  $1$  may consist essentially of the first yarn  $100$  and the second yarn  $200$ . The



## 11

ments, the warp knit construction 10 may comprise the second yarn 200 in an amount ranging from about 3 wt. % to about 5 wt. %—including all amounts and sub-ranges there-between—based on the total weight of the warp knit construction 10.

In a non-limiting example, the second yarn 200 may be present in an amount of about 1 wt. % based on the total weight of the warp knit construction 10. In a non-limiting example, the second yarn 200 may be present in an amount of about 2 wt. % based on the total weight of the warp knit construction 10. In a non-limiting example, the second yarn 200 may be present in an amount of about 3 wt. % based on the total weight of the warp knit construction 10. In a non-limiting example, the second yarn 200 may be present in an amount of about 4 wt. % based on the total weight of the warp knit construction 10. In a non-limiting example, the second yarn 200 may be present in an amount of about 5 wt. % based on the total weight of the warp knit construction 10. In a non-limiting example, the second yarn 200 may be present in an amount of about 6 wt. % based on the total weight of the warp knit construction 10. In a non-limiting example, the second yarn 200 may be present in an amount of about 7 wt. % based on the total weight of the warp knit construction 10. In a non-limiting example, the second yarn 200 may be present in an amount of about 8 wt. % based on the total weight of the warp knit construction 10. In a non-limiting example, the second yarn 200 may be present in an amount of about 9 wt. % based on the total weight of the warp knit construction 10. In a non-limiting example, the second yarn 200 may be present in an amount of about 10 wt. % based on the total weight of the warp knit construction 10.

The fabric 1 may comprise the second yarn 200 in an amount ranging from about 1 wt. % to about 15 wt. %—including all amounts and sub-ranges there-between—based on the total weight of the fabric 1. In some embodiments, the fabric 1 may comprise the second yarn 200 in an amount ranging from about 1 wt. % to about 10 wt. %—including all amounts and sub-ranges there-between—based on the total weight of the fabric 1. In some embodiments, the fabric 1 may comprise the second yarn 200 in an amount ranging from about 2 wt. % to about 9 wt. %—including all amounts and sub-ranges there-between—based on the total weight of the fabric 1. In some embodiments, the fabric 1 may comprise the second yarn 200 in an amount ranging from about 2 wt. % to about 8 wt. %—including all amounts and sub-ranges there-between—based on the total weight of the fabric 1. In some embodiments, the fabric 1 may comprise the second yarn 200 in an amount ranging from about 2 wt. % to about 7 wt. %—including all amounts and sub-ranges there-between—based on the total weight of the fabric 1. In some embodiments, the fabric 1 may comprise the second yarn 200 in an amount ranging from about 3 wt. % to about 6 wt. %—including all amounts and sub-ranges there-between—based on the total weight of the fabric 1. In some embodiments, the fabric 1 may comprise the second yarn 200 in an amount ranging from about 3 wt. % to about 5 wt. %—including all amounts and sub-ranges there-between—based on the total weight of the fabric 1.

In a non-limiting example, the second yarn 200 may be present in an amount of about 1 wt. % based on the total weight of the fabric 1. In a non-limiting example, the second yarn 200 may be present in an amount of about 2 wt. % based on the total weight of the fabric 1. In a non-limiting example, the second yarn 200 may be present in an amount of about 3 wt. % based on the total weight of the fabric 1. In a non-limiting example, the second yarn 200 may be

## 12

present in an amount of about 4 wt. % based on the total weight of the fabric 1. In a non-limiting example, the second yarn 200 may be present in an amount of about 5 wt. % based on the total weight of the fabric 1. In a non-limiting example, the second yarn 200 may be present in an amount of about 6 wt. % based on the total weight of the fabric 1. In a non-limiting example, the second yarn 200 may be present in an amount of about 7 wt. % based on the total weight of the fabric 1. In a non-limiting example, the second yarn 200 may be present in an amount of about 8 wt. % based on the total weight of the fabric 1. In a non-limiting example, the second yarn 200 may be present in an amount of about 9 wt. % based on the total weight of the fabric 1. In a non-limiting example, the second yarn 200 may be present in an amount of about 10 wt. % based on the total weight of the fabric 1.

The first yarn 100 may include natural yarn, synthetic yarn, and combinations thereof. Non-limiting examples of natural yarn include cotton, wool, rayon, and combinations thereof. Non-limiting examples of synthetic yarn include polyester, polyamide (i.e., nylon), polypropylene, viscose, acetate, and combinations thereof. Non-limiting examples of hard yarn include natural-synthetic blends, such as polyester-cotton blend. Non-limiting examples of elastic yarn include polyurethane, such as a thermoplastic polyurethane. Non-limiting examples of polyurethane may further include polyurethane-urea polymer, such as Spandex.

The first yarn 100 may not be a bicomponent yarn. The first yarn 100 may be substantially free of bicomponent yarns. The first yarn 100 may be substantially free of core-sheath yarn. The first yarn 100 may have a first denier. The first denier may range from about 20 to about 150—including all deniers and sub-ranges there-between. In some embodiments, the first denier may range from about 30 to about 120—including all deniers and sub-ranges there-between. In some embodiments, the first denier may range from about 40 to about 100—including all deniers and sub-ranges there-between. In a non-limiting embodiment, the first denier may be about 70.

In some embodiments, the first yarn 100 may comprise a plurality of first yarns that each have a different denier and formed of a variety of natural yarn, synthetic yarn, and combinations thereof—so long as the denier falls within the first denier range and the yarn type fall within the listed natural yarn, synthetic yarn, or combination yarn as described for the first yarn 100.

The second yarn 200 may not be a bicomponent yarn. The second yarn 200 may be substantially free of bicomponent yarn. The second yarn 200 may be substantially free of core-sheath yarn. The second yarn 200 may have a second denier. The second denier may range from about 205 to about 475—including all deniers and sub-ranges there-between. In some embodiments, the second denier may range from about 210 to about 460—including all deniers and sub-ranges there-between. In some embodiments, the second denier may range from about 210 to about 450—including all deniers and sub-ranges there-between. In some embodiments, the second denier may range from about 210 to about 440—including all deniers and sub-ranges there-between. In some embodiments, the second denier may range from about 210 to about 420—including all deniers and sub-ranges there-between.

In a non-limiting embodiment, the second denier may be about 210. In a non-limiting embodiment, the second denier may be about 240. In a non-limiting embodiment, the second denier may be about 280.

In some embodiments, the second denier may range from about 240 to about 475—including all deniers and sub-ranges there-between. In some embodiments, the second denier may range from about 240 to about 460—including all deniers and sub-ranges there-between. In some embodiments, the second denier may range from about 300 to about 440—including all deniers and sub-ranges there-between. In a non-limiting embodiment, the second denier may be about 420.

In some embodiments, the second yarn **200** may be formed of a single yarn having a single sized denier that falls within the second denier range and formed of a single type of elastomeric yarn. In other embodiments, the second yarn **200** may comprise a plurality of second yarns that each have a different denier—so long as the denier falls within the second denier range. In a non-limiting example, the second yarn may comprise two, three, four, five, six, seven, eight, nine, and ten different second yarns—each having a different denier that falls within the second denier range.

In a non-limiting example, the second yarn **200** may include a first portion and a second portion of the second yarn **200**, whereby each thread of the first portion of the second yarn **200** has a denier falling within the second denier range and each thread of the second portion of the second yarn **200** has a denier falling within the second denier range, whereby the denier of the first portion of the second yarn **200** and the denier of the second portion of the second yarn **200** is different.

In a non-limiting example, the second yarn **200** may include a first portion, a second portion, and a third portion of the second yarn **200**, whereby each thread of the first portion of the second yarn **200** has a denier falling within the second denier range, each thread of the second portion of the second yarn **200** has a denier falling within the second denier range, and each thread of the third portion of the second yarn **200** has a denier falling within the second denier range, and whereby the denier of the first portion of the second yarn **200**, the denier of the second portion of the second yarn **200**, and the denier of the third portion of the second yarn **200** is different.

In a non-limiting example, the second yarn **200** may include a first portion, a second portion, a third portion, and a fourth portion of the second yarn **200**, whereby each thread of the first portion of the second yarn **200** has a denier falling within the second denier range, each thread of the second portion of the second yarn **200** has a denier falling within the second denier range, each thread of the third portion of the second yarn **200** has a denier falling within the second denier range, and each thread of the fourth portion of the second yarn **200** has a denier falling within the second denier range, and whereby the denier of the first portion of the second yarn **200**, the denier of the second portion of the second yarn **200**, the denier of the third portion of the second yarn **200**, and the denier of the fourth portion of the second yarn **200** is different.

The warp knit construction **10** may be formed from the first yarn having the first denier and the second yarn having the second denier, whereby a ratio of the second denier to the first denier ranges from about 2:1 to about 16:1—including all ratios and sub-ranges there-between.

In some embodiments, the warp knit construction **10** may be formed from the first yarn having the first denier and the second yarn having the second denier, whereby a ratio of the second denier to the first denier ranges from about 2:1 to about 15:1—including all ratios and sub-ranges there-between. In some embodiments, the warp knit construction **10** may be formed from the first yarn having the first denier and

the second yarn having the second denier, whereby a ratio of the second denier to the first denier ranges from about 6:1 to about 16:1—including all ratios and sub-ranges there-between. In some embodiments, the ratio of the second denier to the first denier ranges from about 5:1 to about 15:1—including all ratios and sub-ranges there-between. In some embodiments, the ratio of the second denier to the first denier ranges from about 7:1 to about 15:1—including all ratios and sub-ranges there-between. In some embodiments, the ratio of the second denier to the first denier ranges from about 8:1 to about 14:1—including all ratios and sub-ranges there-between. In some embodiments, the ratio of the second denier to the first denier ranges from about 9:1 to about 13:1—including all ratios and sub-ranges there-between. In some embodiments, the ratio of the second denier to the first denier ranges from about 10:1 to about 12:1—including all ratios and sub-ranges there-between. In some embodiments, the ratio of the second denier to the first denier ranges from about 10:1 to about 11:1—including all ratios and sub-ranges there-between. In a non-limiting example, the ratio of the second denier to the first denier is about 10.5:1.

It has been discovered that the knitted combination of the first yarn **100** at the first denier and the second yarn **200** at the second denier in the warp knit construction **10**, whereby the first yarn **100** and the second yarn **200** are present in the aforementioned amounts and/or ratios results in a fabric **1** that exhibits a superior resistance to chemical degradation without sacrificing to the longevity of recovery performance necessary for a stretch fabrics.

It has been discovered that the knitted combination of the first yarn **100** forming a plurality of stitches and the second yarn **200** forming a repeating array of cells, whereby the number of stitches present in each cell ranges from 20 to 300 results in a fabric **1** that exhibits a superior resistance to chemical degradation without sacrificing to the longevity of recovery performance necessary for a stretch fabrics.

It has been discovered that the knitted combination of the first yarn **100** having a first denier ranging from about 20 to about 150 and a second yarn **200** in-laid through the first yarn **100**, the second yarn having a second denier ranging from about 240 to about 450, whereby the first yarn **100** is present in an amount ranging from about 90 wt. % to about 99 wt. % and the second yarn is present in an amount ranging from about 1 wt. % to about 10 wt. % results in a fabric **1** that exhibits a superior resistance to chemical degradation without sacrificing to the longevity of recovery performance necessary for a stretch fabrics.

Stretch fabrics have many applications in active wear, which expose these materials to conditions that may not be suitable for prolonged deformation and recovery in such stretch fabrics—such as chlorinated pools. Therefore, a need exists for a new stretch fabric that is suitable for such active wear applications, and which can exhibit the necessary prolonged recovery characteristics that are needed for such applications.

Each of the first yarn **100** and the second yarn **200** of the present invention may be color-dyed.

The fabric **1** of the present invention may be used in the manufacture a textile article. The term ‘textile article’ includes, for example, a garment or article of clothing such as a shirt, pants, skirt, jacket, coat, work shirt, work pants, uniform, outerwear, sportswear, Swimsuit, bra, socks, and underwear, and also includes accessories Such as belts, gloves, mittens, hats, hosiery, or footwear. The term ‘textile article’ may also include such items as sheets, pillowcases, bedspreads, quilts, blankets, comforters, comforter covers, sleeping bags, shower curtains, curtains, drapes, tablecloths,

napkins, wiping cloths, dish towels, and protective coverings for upholstery or furniture.

Examples

The following examples demonstrate the unexpected improvement in chemical degradation resistance for warp knit fabrics.

TABLE 1

|                  | Ex. 1    | Ex. 2    | Ex. 3    | Comp. Ex. 1 |
|------------------|----------|----------|----------|-------------|
| Spandex Content  | 4 wt. %  | 8 wt. %  | 6 wt. %  | 54 wt. %    |
| Spandex Denier   | 420      | 280      | 210      | 140         |
| Nylon Content    | 96 wt. % | 92 wt. % | 94 wt. % | 46 wt. %    |
| Nylon Denier     | 70       | 100 ± 30 | 100 ± 30 | 40          |
| Knit Type        | Rachel   | Rachel   | Rachel   | Tricot      |
| Original Modulus | 0.38     | 0.74     | 1.05     | 3.37        |
| 3x Wet/Dry       | 0.39     | 0.78     | 1.02     | 3.18        |
| Modulus at 30%   |          |          |          |             |
| 6x Wet/Dry       | 0.3      | 0.70     | 1.06     | 3.12        |
| Modulus at 30%   |          |          |          |             |
| 9x Wet/Dry       | 0.37     | 0.76     | 1.05     | 2.98        |
| Modulus at 30%   |          |          |          |             |
| 12x Wet/Dry      | 0.38     | 0.63     | 1.13     | 3.03        |
| Modulus at 30%   |          |          |          |             |
| 15x Wet/Dry      | 0.34     | 0.59     | 1.16     | 3.01        |
| Modulus at 30%   |          |          |          |             |
| 18x Wet/Dry      | 0.38     | 0.66     | 1.10     | 2.88        |
| Modulus at 30%   |          |          |          |             |
| 21x Wet/Dry      | 0.39     | 0.78     | 1.05     | 2.76        |
| Modulus at 30%   |          |          |          |             |
| % Modulus Change | 3%       | 5%       | 0%       | -18%        |

Comp. Ex. 2 Comp. Ex. 3 Comp. Ex. 4 Comp. Ex. 5

|                  |          |          |          |          |
|------------------|----------|----------|----------|----------|
| Spandex Content  | 38 wt. % | 24 wt. % | 20 wt. % | 20 wt. % |
| Spandex Denier   | 105      | 70       | 40       | 40       |
| Nylon Content    | 62 wt. % | 76 wt. % | 80 wt. % | 80 wt. % |
| Nylon Denier     | 40       | 45       | 70       | 70       |
| Knit Type        | Tricot   | Tricot   | Tricot   | Tricot   |
| Original Modulus | 1.94     | 1.21     | 0.61     | 0.43     |
| 3x Wet/Dry       | 1.66     | 1.07     | 0.4      | 0.31     |
| Modulus at 30%   |          |          |          |          |
| 6x Wet/Dry       | 1.63     | 1.01     | 0.3      | 0.29     |
| Modulus at 30%   |          |          |          |          |
| 9x Wet/Dry       | 1.57     | 0.95     | 0.17     | 0.2      |
| Modulus at 30%   |          |          |          |          |
| 12x Wet/Dry      | 1.57     | 0.98     | 0.17     | 0.22     |
| Modulus at 30%   |          |          |          |          |
| 15x Wet/Dry      | 1.54     | 0.96     | 0.12     | 0.18     |
| Modulus at 30%   |          |          |          |          |
| 18x Wet/Dry      | 1.45     | 0.88     | 0.15     | 0.2      |
| Modulus at 30%   |          |          |          |          |
| 21x Wet/Dry      | 1.41     | 0.84     | 0.11     | 0.16     |
| Modulus at 30%   |          |          |          |          |
| % Modulus Change | -27%     | -31%     | -82%     | -63%     |

Comp. Ex. 6 Comp. Ex. 7

|                  |          |          |
|------------------|----------|----------|
| Spandex Content  | 20 wt. % | 19 wt. % |
| Spandex Denier   | 40       | 40       |
| Nylon Content    | 80 wt. % | 81 wt. % |
| Nylon Denier     | 70       | 40       |
| Knit Type        | Tricot   | Tricot   |
| Original Modulus | 1.73     | 0.72     |
| 3x Wet/Dry       | 1.58     | 0.46     |
| Modulus at 30%   |          |          |
| 6x Wet/Dry       | 1.54     | 0.45     |
| Modulus at 30%   |          |          |
| 9x Wet/Dry       | 1.45     | 0.39     |
| Modulus at 30%   |          |          |
| 12x Wet/Dry      | 1.5      | 0.43     |
| Modulus at 30%   |          |          |
| 15x Wet/Dry      | 1.37     | 0.42     |
| Modulus at 30%   |          |          |
| 18x Wet/Dry      | 1.39     | 0.30     |

TABLE 1-continued

|                  |      |      |
|------------------|------|------|
| Modulus at 30%   | 1.48 | 0.31 |
| 21x Wet/Dry      |      |      |
| Modulus at 30%   |      |      |
| % Modulus Change | -15% | 57%  |

Each test sample fabric of Examples 1-3 and Comparative Examples 1-7 underwent a wet/dry modulus test, whereby each sample was exposed to a number of wet-cycles using chlorine containing water to simulate a swimming pool environment. The swimming pool environment included chlorine in an amount of 5 ppm and an alkalinity of 80 ppm at a pH of 7.5.

As demonstrated by Table 1, the combination of using a Rachel knit pattern with a hard yarn having a denier ranging from 70 to 130 and an elastomeric yarn having a denier ranging from 210 to 420 provided for a surprising improvement in the resistance to change in modulus after repeated wet-cycles as compared to fabrics with elastomeric yarn having a denier under 210. In particular, each of the inventive fabrics demonstrated a change in modulus that is 5% or less—whereas the comparative fabrics were at least 15% or more in the change in modulus.

Additionally, although not shown a fabric was not able to be formed using tricot pattern and with a hard yarn having a denier of 70 and an elastomeric yarn having a denier ranging from 210 to 420.

What is claimed is:

1. A fabric having a warp knit construction comprising: a repeating array of cells, each cell defined by an inlay yarn; a plurality of stiches formed inside of each cell, the plurality of stiches formed by a hard yarn having a denier ranging from about 20 to about 130 denier; and wherein the number of stiches per cell ranges from about 20 to about 300; and wherein the inlay yarn comprises an elastomeric yarn having a denier ranging from about 210 to about 420; and wherein the warp knit construction is a raschel knit; and wherein the inlay yarn is present in an amount ranging from about 1 wt. % to about 10 wt. % based on the total weight of the fabric, and wherein the hard yarn is present in an amount ranging from about 90 wt. % to about 99 wt. % based on the total weight of the fabric.
2. The fabric according to claim 1, wherein the elastomeric yarn selected from spandex yarn, rubber yarn, and thermoplastic polyurethane yarn.
3. The fabric according to claim 1, wherein the elastomeric yarn is not a bicomponent yarn, and wherein the hard yarn is not a bicomponent yarn.
4. The fabric according to claim 1, wherein the hard yarn is selected from the group consisting of polyester, polyamide, polypropylene, cotton, rayon, polyester-cotton blend.
5. The fabric according to claim 1, wherein each of the cells is defined by a closed perimeter that is formed by the inlay yarn.
6. The fabric according to claim 5, wherein the closed perimeter of each cell spans at least 5 wales in the warp knit construction, and wherein the closed perimeter of each cell spans at least 5 courses in the warp knit construction.
7. A fabric having a warp knit construction comprising: a first yarn forming a plurality of stiches extending along in a knit direction, the first yarn comprising a hard yarn having a first denier ranging from about 20 to about 70;

## 17

a second yarn in-laid through the first yarn, the second yarn extending along the knit direction and having a repeating pattern that extends across at least 4 wales for every 4 courses, the second yarn having a second denier; and

wherein a ratio of the second denier to the first denier ranges from about 2:1 to about 15:1.

8. The fabric according to claim 7, wherein the repeating pattern of the second yarn extends across at least 5 wales for every 5 courses.

9. The fabric according to claim 7, wherein the second denier ranges from about 210 to about 450.

10. The fabric according to claim 7, wherein the second yarn is selected from spandex yarn, rubber yarn, and thermoplastic polyurethane yarn.

11. The fabric according to claim 7, wherein the second yarn is present in an amount ranging from about 1 wt. % to about 10 wt. % based on the total weight of the fabric, and wherein the first yarn is present in an amount ranging from about 90 wt. % to about 99 wt. % based on the total weight of the fabric.

12. The fabric according to claim 7, wherein the warp knit construction is a raschel knit.

13. A fabric having a warp knit construction comprising: a first yarn forming a plurality of stitches, the first yarn being a hard yarn and having a first denier ranging from about 20 to about 150; a second yarn in-laid through the first yarn, the second yarn being an elastomeric yarn and having a second denier ranging from about 210 to about 450; and

## 18

wherein the first yarn is present in an amount ranging from about 90 wt. % to about 99 wt. % based on the total weight of the fabric, and wherein the second yarn is present in an amount ranging from about 1 wt. % to about 10 wt. % based on the total weight of the fabric.

14. The fabric according to claim 13, wherein the first yarn is not a bicomponent yarn, and wherein the second yarn is not a bicomponent yarn.

15. The fabric according to claim 13, wherein the warp knit construction is a raschel knit.

16. The fabric according to claim 1, wherein the denier of the hard yarn ranges from about 20 to about 70.

17. The fabric according to claim 7, wherein the hard yarn comprises a first hard yarn and a second hard yarn, wherein the first denier of the first hard yarn is different from the first denier of the second hard yarn.

18. The fabric according to claim 13, wherein the hard yarn comprises a first hard yarn and a second hard yarn, wherein the first denier of the first hard yarn is different from the first denier of the second hard yarn.

19. The fabric according to claim 18, wherein the first denier of the first hard yarn is about 70 and the first denier of the second hard yarn is about 30.

20. The fabric according to claim 13, wherein the hard yarn comprises a first hard yarn and a second hard yarn, wherein the first hard yarn comprises nylon and the second hard yarn comprises one or more of polyester and nylon.

\* \* \* \* \*